

# UNITED STATES PATENT OFFICE.

WENDELL R. SWINT, OF WILMINGTON, DELAWARE, ASSIGNOR TO E. I. DU PONT DE NEMOURS AND COMPANY, OF WILMINGTON, DELAWARE, A CORPORATION OF DELAWARE.

## EXPLOSIVE COMPOSITION.

1,307,766.

Specification of Letters Patent. Patented June 24, 1919.

No Drawing.

Application filed January 31, 1918. Serial No. 214,637.

To all whom it may concern:

Be it known that I, WENDELL R. SWINT, of Wilmington, in the county of New Castle, and in the State of Delaware, have invented 5 a certain new and useful Improvement in Explosive Compositions, and do hereby declare that the following is a full, clear, and exact description thereof.

My invention relates particularly to the 10 production of high explosives having advantageous characteristics, and more particularly to dynamites formed by the use of highly nitrated cellulose.

The object of my invention is to provide 15 explosive compositions in the nature of dynamites containing highly nitrated cellulose.

A further object of my invention is to provide 20 compositions of this character containing nitroglycerin.

The object of my invention is further to provide 25 explosive compositions having the following advantageous characteristics:— Compositions of this character provide dy-

namites that are cheaper to produce than dynamites previously produced without changing the quality. Furthermore, compositions made in accordance with my invention are detonatable and can be used in 30 blasting.

Further objects of my invention will appear from the detailed description thereof contained hereinafter.

While my invention is capable of embodiment in many different forms, for the 35 purpose of illustration I shall describe only certain forms of my invention hereinafter.

Compositions made in accordance with my invention and which contain nitrocellulose 40 of a high degree of nitration, as for example nitrocellulose containing approximately 13% or more of nitrogen, can be used with the above advantageous results and can be made with or without the presence of nitrocellulose having a lower degree of nitration. The nitrocellulose having a lower degree of nitration acts to gelatinize the composition containing the nitrocellulose having a high degree of nitration. Such nitrocellulose having a lower degree of nitration might contain approximately 12.25% nitrogen.

Furthermore, compositions made in ac-

cordance with my invention may contain an oxygen-carrying salt, as for example sodium or potassium nitrate or barium nitrate. 55

Again, they may contain combustible material, such for example as wood pulp, to act as an absorbent.

As such examples of my invention, I may provide compositions containing the following constituents:—

|                                            |     |
|--------------------------------------------|-----|
| Nitroglycerin                              | 30% |
| Insoluble nitrocellulose of high nitration | 10% |
| Sodium nitrate                             | 55% |
| Wood pulp                                  | 5%  |

Another example would be:—

|                                            |       |
|--------------------------------------------|-------|
| Nitroglycerin                              | 40 %. |
| Insoluble nitrocellulose of high nitration | 12.1% |
| Soluble nitrocellulose of lower nitration  | 0.9%. |
| Sodium nitrate                             | 43.0% |
| Wood pulp                                  | 4.0%  |

It will be understood that, in the above compositions, however, the oxygen-carrying salt and the absorbent may be omitted, and that other ingredients may be added to any 80 of the aforesaid compositions.

While I have described my invention above in detail, I wish it to be understood that many changes may be made therein without departing from the spirit of the invention. 85

I claim:—

1. A high explosive composition containing nitrocellulose of a high degree of nitration, nitroglycerin, and wood pulp. 90

2. An explosive composition containing nitrocellulose of a high degree of nitration, nitroglycerin, nitrocellulose of a lower degree of nitration, and wood pulp.

3. An explosive composition containing nitrocellulose of a high degree of nitration, nitroglycerin, an oxygen-carrying salt, and wood pulp. 95

4. An explosive composition containing nitrocellulose of a high degree of nitration, nitroglycerin, nitrocellulose of a lower degree of nitration, an oxygen-carrying salt, and wood pulp. 100

5. An explosive composition containing

nitrocellulose of a high degree of nitration, nitroglycerin, sodium nitrate, and wood pulp.

6. An explosive composition containing  
5 nitrocellulose of a high degree of nitration, nitroglycerin, nitrocellulose of a lower degree of nitration, sodium nitrate and wood pulp.

In testimony that I claim the foregoing I have hereunto set my hand.

WENDELL R. SWINT.

Witnesses:

P. E. STRICKLAND,  
H. L. BRADLEY.

Copies of this patent may be obtained for five cents each, by addressing the "Commissioner of Patents, Washington, D. C."